

## UNITED STATES PATENT OFFICE

2,514,019

## PROCESS FOR PRODUCING A PLASTIC COMPOSITION FOR BATTERY BOXES

Cecil B. Wilde, Compton, Calif., assignor to Stauffer Chemical Company, a corporation of California

No Drawing. Application July 6, 1948,  
Serial No. 37,309

3 Claims. (Cl. 106—202)

1

This invention relates to plastic compositions and particularly to those which are impervious to water, resistant to the action of sulfuric acid of the strength usually employed in storage batteries and which, when molded, are capable of retaining their character under ordinary thermal conditions.

It is well known that, in the fabrication of battery boxes and like articles which, in use, are subjected to the action of sulfuric acid and which are required to have both mechanical and dielectric strength, it is necessary to utilize materials which are at least partially unaffected by the acid. A typical composition as used heretofore has consisted of a mixture of a suitable hydrocarbon such as asphalt or other bitumen, a filler such as diatomaceous earth or the like, and asbestos fibres. This material has been prepared by first melting the hydrocarbon and placing it in a mixer together with the fibrous material and the filling material. Because of the necessity of employing a hydrocarbon material which has inherently a relatively high softening point, the mixing of the hydrocarbon and fibrous material must be at a relatively high temperature. To secure adequate mixing, the mixing operation must be continued for a relatively long period of time. As a consequence, the fibres become broken and the tensile strength of the ultimate product is affected adversely; if a vegetable fibre is employed, it is scorched, charred or at least lowered materially in strength. Further, it is difficult to distribute the fibrous material through the sticky, plastic mass of hydrocarbon and, as a consequence, the mixing must be continued for an inordinately long period of time or else the mixture is not homogeneous. In either case, the properties of the substance are affected adversely with respect to such characteristics as tensile strength, dielectric strength, acid resistance and uniformity. Such a process as I have described is disclosed in Patent 1,752,917.

It has also been proposed in Patent 1,892,703 to mix the three constituents in the dry state and then apply heat. This process provides some improvement over that previously described. However, while the dry mix may be homogeneous, this is not always true of the mass after heating, for apparently the hydrocarbon

does not bond to the fibrous filler when the heat is applied and the fibres are not impregnated to the desired extent. Increasing the degrees of heating merely scorches the fibre.

5 In accordance with the present invention, I prepare each of the constituents of the mixture separately, grinding the hydrocarbon material to finely divided form, for example, so that at least 80% of the hydrocarbon will pass a 40 mesh screen; the fibrous material, which has been previously placed in shredded form while dry, is fluffed so that the material is of relatively low density. The filler is also in finely divided form, for example, so that all of it will pass a 100 mesh screen. The hydrocarbon material usually comprises from 45% to 55% of the mixture and the earth from 25% to 45%. The three constituents are then mixed in a suitable mixing device, such as a paddle mixer, to form a homogeneous mass 10 of the three. Thus, the hydrocarbon material is fairly distributed throughout the fibrous material and the earth, and the fibres are uniformly coated with the earth and hydrocarbon material without destroying the individual fibres 15 or reducing their length. During the course of the mixing operation, about 10% by weight of water is added to the mixture undergoing mixing. This facilitates deposit of the finely divided earth and hydrocarbon on the fibres. The 20 quantity of water added should be between 5% and 20% by weight of the mass; this quantity of water is insufficient to make the mass wet or soggy; in fact, a visual examination of the material issuing from the mixer will fail to reveal 25 the presence of the water and the mixture can be squeezed or pressed in the hand without obtaining any evidence of the presence of water. The mixture is then passed through a steam heated screw masticator extruder or equivalent 30 device, wherein the mixture is heated to a temperature of 250° to 325° F. In the masticator extruder, the mixture is worked and kneaded together; the material issuing from the mixer is 35 homogeneous, the hydrocarbon having been melted so that the earth and fibre are uniformly coated and impregnated. The presence 40 of the water facilitates this; at the same time, if a vegetable fibre or a mixture of these is employed, the fibre is protected against burning or 45 scorching or lowering of the fibre strength. Due

to the pressure exerted upon the mixture in the masticator extruder, the water present is converted into steam which facilitates the uniform heating of the mixture and insures that the material issuing from the masticator extruder is uniform with all of the hydrocarbon melted and impregnating or coating the fibre, the individual fibres of which are not broken or reduced in length. The material is then preferably exposed to the atmosphere for a period of from 1 to 4 minutes to permit the mass to steam freely; during the free steaming period, the mass is subject to additional heating by means of radiant heaters disposed closely adjacent to the mass of material; a convenient manner of obtaining this is to move the stream of material issuing from the masticator extruder along on a conveyor beneath suitable radiant heaters. This permits any excess water vapor present as steam to issue from the material. The material is then again preferably kneaded in a second masticator for a short period of time to provide further uniformity in the mixture. The material is then ready for processing in the usual manner in a suitable press to form a battery box or like article.

The usual fibres employed heretofore have generally been asbestos or cotton linters; both are relatively expensive. I have found that I can utilize other vegetable fibres alone or mixed together in place of cotton or in addition to cotton, such as kraft, sulfite or like fibres. These are used in an amount up to about 20% of the mixture and preferably 10%-12% by weight of the mixture. The use of such fibres is made possible because of the absence of high temperature conditions and long mixing periods which either destroy the fibre length or reduce its strength objectionably, or both.

*Example 1*

As illustrative of the practice of the present invention, 52 parts of an asphalt having a ball and ring softening point of 275° F. and a penetration of 13 @ 115° F. and ground to minus 40 mesh were mixed with 11 parts of kraft pulp obtained by shredding used kraft paper bags together with 37 parts of diatomaceous earth, all minus 100 mesh. The three materials were uniformly mixed in a dry mixer, 5%-20% by weight of the mixture of water being added during the course of the mixing operation. The mixture was then passed to a masticator extruder to a temperature of 250°-325° F., wherein the material was heated until the asphalt had melted and uniformly impregnated the earth and fibre. The mixture was then permitted to steam freely while heated by radiant heat for two minutes, so that no loss of temperature occurred. After this, it was kneaded for two to four minutes when it was ready for formation into a typical battery box in a press and in the well known manner. The composition, when molded in this manner had the following characteristics:

Tensile strength 1352 pounds per square in.  
Percent elongation 1.9%  
Impact 0.50 foot pound

Bulge test:

Side 0.069 inch  
End 0.205 inch

*Example 2*

The procedure outlined under Example 1 was followed, but equal parts by weight of cotton

linters and shredded kraft pulp were employed instead of the kraft pulp. The battery box had the following characteristics:

Tensile strength 1443 pounds per square in.  
Percent elongation 1.96%  
Impact strength 0.50 foot pound

Bulge test:

Side 0.063 inch  
End 0.150 inch

*Example 3*

The procedure outlined under Example 1 was followed utilizing 12% of dry, fluffed, shredded sulfite pulp. The battery box which was formed was of acceptable characteristics and properties.

*Example 4*

The procedure outlined under Example 1 was followed, but equal parts by weight of cotton linters and shredded sulfite pulp were employed. The battery box which was formed was of acceptable characteristics and properties.

*Example 5*

The procedure outlined under Example 1 was followed, but equal parts by weight of cotton linters, shredded sulfite pulp, and shredded kraft pulp were employed. The battery box which was formed was of acceptable characteristics and properties.

I claim:

1. A process for producing a plastic composition for battery boxes comprising mixing together in a dry state and substantially at a normal atmospheric temperature a bitumen in the form of a dry, finely divided solid, a finely divided earth, and a pre-fluffed dry fibrous material of low density and selected from the group consisting of kraft pulp, sulfite pulp and mixtures thereof with cotton linters, the mixture containing from 45% to 55% of the bitumen, from 25% to 45% of the earth, and from 10% to 20% of the fibrous material, adding to the mixture during the mixing from 5% to 20% of water and continuing the mixing until a dry homogeneous mixture is formed, and thereafter heating the mixture to a temperature of from 250° F. to 325° F. while kneading the material under pressure until the bitumen is melted in the mixture and the mixture is substantially free of water.

2. A process for producing a plastic composition for battery boxes comprising mixing together a dry finely divided bitumen, a finely divided earth, and a dry fibrous pre-fluffed material selected from the group consisting of kraft pulp, sulfite pulp and mixtures thereof with cotton linters, the mixture containing from 45%

to 55% of the bitumen, from 25% to 45% of the earth, and from 10% to 20% of the fibrous material, the mixing being at a temperature whereat the bitumen is a solid, adding to the mixture during the mixing from 5% to 20% of water and continuing the mixing until a dry homogeneous mixture is formed, and then heating the mixture to a temperature of from 250° F. to 325° F. while kneading the material under pressure until the bitumen is melted in the mixture and the mixture is substantially free of water.

3. A process for producing a plastic composition for battery boxes comprising mixing together a dry finely divided solid bitumen of which at least 80% will pass a 40 mesh screen, a

finely divided earth, and a dry pre-fluffed fibrous material selected from the group consisting of kraft pulp, sulfite pulp and mixtures thereof with cotton linters, the mixture containing from 45% to 55% of the bitumen, from 25% to 45% of the earth, and from 10% to 20% of the fibrous material, adding to the mixture during the mixing from 5% to 20% of water and continuing the mixing until a dry homogeneous mixture is formed, and then heating the mixture to a temperature of from 250° F. to 325° F. while kneading the material under pressure until the bitumen is melted in the mixture and the mixture is dry.

CECIL B. WILDE.

## REFERENCES CITED

The following references are of record in the file of this patent:

## UNITED STATES PATENTS

| Number    | Name    | Date          |
|-----------|---------|---------------|
| 337,472   | Allen   | Mar. 9, 1886  |
| 1,156,122 | Woodley | Oct. 12, 1915 |
| 1,751,690 | Faben   | Mar. 25, 1930 |
| 1,771,643 | Lukens  | July 29, 1930 |
| 1,892,703 | Lindh   | Jan. 3, 1933  |
| 2,023,675 | Fischer | Dec. 10, 1935 |